# EUROPEAN PATENT SPECIFICATION

(11) **EP 0 843 149 B1**
(45) Date of publication and mention of the grant of the patent: **26.08.1998**
(21) Application number: 96308166.6
(22) Date of filing: 12.11.1996
(51) Int. Cl.: F41H 5/04

(54) **Composite armor panel and manufacturing method therefor**
Verbundpanzerplatte und Verfahren zur Herstellung
Plaque de blindage composite et son procédé de fabrication

(43) Date of publication of application: 20.05.1998
(73) Proprietor: MOFET ETZION, North Yehuda 90200 (IL)
(72) Inventor: Cohen, Michael, Mobile Post North Yehuda 90200 (IL); Israeli, Avinoam, Mobile Post North Yehuda 90200 (IL)
(74) Representative: Goodanew, Martin Eric

(56) References cited:
- DE-A- 3 228 264
- DE-A- 3 507 216
- FR-A- 1 566 448
- FR-A- 2 559 254
- FR-A- 2 711 782
- GB-A- 1 081 464
- GB-A- 1 352 418
- GB-A- 2 272 272
- US-A- 3 705 558
- US-A- 4 061 815
- US-A- 5 361 678

## Description

The present invention relates to a composite armor plate. More particularly, the invention provides an armored plate providing lightweight ballistic protection which may be worn by the user, and for protecting light mobile equipment and vehicles against high-speed armor-piercing projectiles or fragments. The invention also relates to multi-layer armor panels incorporating the plate, and methods for manufacturing the plate.

There are three main considerations concerning protective armor plates and panels. The first consideration is weight. Protective armor for heavy but mobile military equipment, such as tanks and large ships, is known. Such armor usually comprises a thick layer of alloy steel, which is intended to provide protection against heavy and explosive projectiles. Due to its weight, such armor is quite unsuitable for light vehicles such as automobiles, jeeps, light boats, or aircraft, whose performance is compromised by steel panels having a thickness of more than a few millimeters.

Armor for light vehicles is expected to prevent penetration of bullets of any weight, even when impacting at a speed in the range of 700 to 1000 meters per second. The maximum armor weight which is acceptable for use on light vehicles varies with the type of vehicle, but generally falls in the range of 40 to 70 kg/m².

A second consideration is cost. Overly complex armor arrangements, particularly those depending entirely on synthetic fibers, can be responsible for a notable proportion of the total vehicle cost, and can make its manufacture non-profitable.

A third consideration in armor design is compactness. A thick armor panel, including air spaces between its various layers, increases the target profile and the wind resistance of the vehicle. In the case of civilian retrofitted armored automobiles which are outfitted with internal armor, there is simply no room for a thick panel in most of the areas requiring protection.

Fairly recent examples of armor systems are described in U.S. Patent No. 4,836,084, disclosing an armor plate composite including a supporting plate consisting of an open honeycomb structure of aluminium; and U.S. Patent No. 4,868,040, disclosing an antiballistic composite armor including a shock-absorbing layer. Also of interest is U.S. Patent 4,529,640, disclosing spaced armor including a hexagonal honeycomb core member.

Other armor plate panels are disclosed, e.g., in British Patents 1,081,464; 1,352,418; 2,272,272, and in U.S. Patent 4,061,815 wherein the use of sintered refractory material, as well as the use of ceramic materials, are described.

Ceramic materials are nonmetallic, inorganic solids having a crystalline or glassy structure, and have many useful physical properties, including resistance to heat, abrasion and compression, high rigidity, low weight in comparison with steel, and outstanding chemical stabiity. Such properties have long drawn the attention of armor designers, and solid ceramic plates, in thicknesses ranging from 3 mm. for personal protection to 50 mm. for heavy military vehicles, are commercially available for such use.

Much research has been devoted to improving the low tensile and low flexible strength and poor fracture toughness of ceramic materials; however, these remain the major drawbacks to the use of ceramic plates and other large components which can crack and/or shatter in response to the shock of an incoming projectile.

A known form of armor plating using ceramics is produced in Israel by cutting 5 mm. steel plates to the sizes required, heat-treating the steel and adding a ceramic coating. One disadvantage of this type of panel is that on completion the panels are almost impossible to modify. In use, the ceramic coating performs well against the first bullet, but tends to shatter, and thus fails to protect against further projectiles.

Light-weight, flexible armored articles of clothing have also been used for many decades, for personal protection against fire-arm projectiles and projectile splinters. Examples of this type of armor are found in U.S. Patent No. 4,090,005. Such clothing is certainly valuable against low-energy projectiles, such as those fired from a distance of several hundred meters, but fails to protect the wearer against high-velocity projectiles originating at closer range. If made to provide such protection, the weight and/or cost of such clothing discourages its use. A further known problem with such clothing is that even when it succeeds in stopping a projectile the user may suffer injury due to indentation of the vest into the body, caused by too small a body area being impacted and required to absorb the energy of a bullet.

A common problem with prior art ceramic armor concerns damage inflicted on the armor structure by a first projectile, whether stopped or penetrating. Such damage weakens the armor panel, and so allows penetration of a following projectile, impacting within a few centimeters of the first.

In French Patent 2,711,782, there is described a steel panel reinforced with ceramic materials. However, due to the rigidity and lack of elasticity of the steel of said panel, said panel does not have the ability to deflect armor-piercing projectiles unless a thickness of about 8-9 mm of steel is used, which makes the panel rather heavy.

U.S. Patent 5,361,678 (basis for the preamble of claim 1) discloses a composite armor plate comprising a closely packed layer of spherical ceramic balls distributed in an aluminium or titanium alloy matrix, the balls being provided with a coating to reduce damage from thermal shock during manufacture of the plate.

U.S. Patent 3,705,558 discloses a lightweight armor plate comprising at least two layers of ceramic balls. The ceramic balls are in contact with each other and leave small gaps for entry of molten metal. In one embodiment, the ceramic balls are encased in a stainless steel wire screen; and in another embodiment, the composite armor is manufactured by adhering nickel-coated alumina spheres to an aluminium alloy plate by means of a polysulfide adhesive. Such an armor plate is difficult to manufacture because the ceramic spheres may be damaged by thermal shock arising from molten metal contact. The ceramic spheres are also sometimes displaced during casting of molten metal into interstices between the spheres.

In order to minimize such displacement, U.S. Patent 4,534,266 and 4,945,814 propose a network of interlinked metal shells to encase ceramic inserts during casting of molten metal. After the metal solidifies, the metal shells are incorporated into the composite armor. It has been determined, however, that such a network of interlinked metal shells substantially increases the overall weight of the armored panel and decreases the stopping power thereof.

In U.S. Patents 3,523,057 and 5,134,725 there are described further armored panels incorporating ceramic balls. However, said panels are flexible and it has been found that the flexibility of said panels substantially reduces their stopping strength upon impact, since the force of impact itself causes a flexing of said panels and a reduction of the supporting effect of adjacent ceramic balls on the impacted ceramic balls.

The present invention is therefore intended to obviate the disadvantages of prior art ceramic armor, and to provide an armor plate which is effective against small-caliber armor-piercing projectiles, yet is of light weight, i.e. having a weight of less than 45 kg/m², which is equivalent to about 9 lbs/ft², and low bulk.

A further object of the invention is to provide an armor panel which is particularly effective in arresting a plurality of projectiles impacting upon the same general area of the panel.

Accordingly, having regard to what is known from US-A-5361678, the invention provides a composite armor plate for absorbing and dissipating kinetic energy from high velocity, armor-piercing projectiles, said plate comprising a single internal layer of high density ceramic pellets which are directly bound and retained in plate form by a solidified material such that the pellets are bound in a plurality of superposed rows and each of a majority of said pellets is in contact with at least four adjacent pellets, characterised in that the pellets have an Al₂ O₃ content of at least 93% and a specific gravity of at least 2.5, the majority of the pellets each have a major axis of a length in the range of from 3 to 12 mm, the solidified material, and hence the plate, is elastic at a temperature below 250°C, and the weight of said plate does not exceed 45 kg/m².

Said solidified material can be any suitable material which is elastic at a temperature below 250°C, such as aluminium or other suitable metal, epoxy, a thermoplastic polymer, or a thermoset plastic. In a preferred embodiment of the present invention, there is provided an armored plate wherein the solidified material contains at least 80% aluminium.

It is further to be noted that the elasticity of the material used in the present invention serves, to a certain extent, to increase the probability that a projectile will simultaneously impact several pellets, thereby increasing the efficiency of the stopping power of the panel of the present invention.

In a further preferred embodiment of the invention, there is provided a multi-layered armor panel, comprising an outer, impact-receiving layer consisting of a composite armor plate as hereinbefore defined for deforming and shattering an impacting high velocity, armor-piercing projectile, and an inner layer adjacent to said outer layer comprising a tough woven textile material for causing an asymmetric deformation of the remaining fragments of said projectile and for absorbing the remaining kinetic energy from said fragments, said inner layer having a thickness of at least 50% of that of said outer, impact-receiving layer, and said panel being adapted to stop three bullets fired sequentially at a triangular area of said panel, the sides of said triangle being 5 cm each.

As will be realized, none of said prior art patents teaches or suggests the surprising and unexpected stopping power of a single layer of ceramic pellets in direct contact with each other which, as will be shown hereinafter, successfully prevents penetration of armor-piercing 7.6 mm calibre AK-47 projectiles despite the light weight of the plate incorporating said pellets.

Thus, it has been found that the novel armor of the present invention traps incoming projectiles between several sphere-like, very hard ceramic pellets which are held in a single layer in rigid mutual relationship. The moderate size of the pellets ensures that the damage caused by a first projectile is localized and does not spread to adjoining areas.

An incoming projectile may contact the pellet array in one of three ways:
**1. Centre contact.** The impact allows the full volume of the pellet to participate in stopping the projectile, which cannot penetrate without pulverising the whole pellet, an energy-intensive task. The pellets used are either spheres or shapes approaching a spherical form, and this form, when supported in a rigid matrix, has been found to be significantly better at resisting shattering than rectangular shapes.
**2. Flank contact.** The impact causes projectile yaw, thus making projectile arrest easier, as a larger frontal area is contacted, and not only the sharp nose of the projectile. The projectile is deflected sideways and needs to form for itself a large aperture to penetrate, thus allowing the armor to absorb the projectile energy.
**3. Valley contact.** The projectile is jammed, usually between the flanks of three pellets, all of which participate in projectile arrest. The high side forces applied to the pellets are resisted by the pellets adjacent thereto as held by the solid matrix, and penetration is prevented. A test was arranged using a laser-aimed AK47 rifle firing an armor-piercing incindiary AK47 7.62mm caliber round manufactured in Russia, to achieve this particular contact mode, and theory confirmation was obtained that such a result is indeed obtained in practice.

During research and development for the present invention, the preparation of a plate-like composite casting was required, wherein ceramic pellets occupied a centre layer and cast aluminium completely embedded the pellets. When using molten metal the pellets would cool the molten metal, and furthermore, the required close pellet formation would be disturbed by the casting process. As mentioned above, this problem was encountered by McDougal in U.S. Patent 3,705,558. An attempt to solve this problem was suggested by Huet in U.S. Patents 4,534,266 and 4,945,814 and Roopchand, et al. in U.S. Patent 5,361,678 suggested a further solution involving coating the ceramic bodies with a binder and ceramic particles, followed by the introduction of the molten metal into the die.

It is therefore a further object of the present invention to provide a method of manufacturing composite armor plate as described herein, without introducing non-essential and extraneous further components into the final panel and thereby to assure direct contact between adjacent pellets.

Thus, the present invention provides a method for producing a composite armor plate as defined hereinabove, comprising providing a mould having a bottom, two major surfaces, two minor surfaces and an open top, wherein the distance between said two major surfaces is from about 1.2 to about 1.8 times the major axis of said pellets; inserting said pellets into said mould to form a plurality of superposed rows of pellets extending substantially along the entire distance between said minor side surfaces, and from said bottom substantially to said open top; incrementally heating said mould and the pellets contained therein to a temperature of at least 100°C above the flow point of the material to be poured in the mould; pouring molten material into said mould to fill the same; allowing said molten material to solidify; and removing said composite armor plate from said mould.

The present invention also provides a method for producing a composite armor plate, comprising providing a mould having a bottom, two major surfaces, two minor surfaces and an open top, wherein the distance between said two major surfaces is from about 1.2 to 1.8 times the major axis of said pellets; inserting said pellets into said mould to form a plurality of superposed rows of pellets extending substantially along the entire distance between said minor side surfaces, and from said bottom substantially to said open top; pouring liquid epoxy resin into said mould to fill the same; allowing said epoxy to solidify; and removing said composite armor plate from said mould.

As will be realized, when preparing the composite armor plate of the present invention, said pellets do not necessarily have to be completely covered on both sides by said solidified material, and they can touch or even bulge from the outer surfaces of the formed panel.

Further embodiments of the invention, including weight-critical armored clothing, will also be described further below.

The invention will now be described in connection with certain preferred embodiments with reference to the following illustrative figures so that it may be more fully understood.

With reference now to the figures in detail, it is stressed that the particulars shown are by way of example and for purposes of illustrative discussion of the preferred embodiments of the present invention only, and are presented in the cause of providing what is believed to be the most useful and readily understood description of the principles and conceptual aspects of the invention. In this regard, no attempt is made to show structural details of the invention in more detail than is necessary for a fundamental understanding of the invention, the description taken with the drawings making apparent to those skilled in the art how the several forms of the invention may be embodied in practice.

In the drawings:
- Fig. 1: is a perspective, fragmented view of a preferred embodiment of an armor panel according to the invention;
- Figs. 2 and 3: are perspective views of further pellet embodiments;
- Fig. 4: is a sectional view of a two-layer embodiment of the armor panel; and
- Fig. 5: is a diagrammatic view of a mould used in the methods for manufacturing the panel.

There is seen in Fig. 1 a composite armor material 10 for absorbing and dissipating kinetic energy from high- velocity projectiles 12. A panel 14 is formed from a solidified material 16, the panel having an internal layer of high-density ceramic pellets 18. The outer faces of the panel are formed from the solidified material 16, and pellets 18 are embedded therein. The nature of the solidified material 16 is selected in accordance with the weight, performance and cost considerations applicable to the intended use of the armor.

Armor for land and sea vehicles is suitably made using a metal casting alloy containing at least 80% aluminum. A suitable alloy is Aluminum Association No. 535.0, which combines a high tensile strength of 35,000 kg/in², with excellent ductility, having 9% elongation. Further suitable alloys are of the type containing 5% silicon B443.0. These alloys are easy to cast in thin sections; their poor machinability is of little concern in the application of the present invention. An epoxy or other plastic or polymeric material, advantageously fiber-reinforced, is also suitable.

Pellets 18 have an alumina (Al₂O₃) content of at least 93%, and have a hardness of 9 on the Mohs scale. Regarding size, the majority of pellets have a major axis in the range of from about 3-12 mm, the preferred range being from 6-10 mm.

There are shown in Fig. 1, for illustrative purposes, a mixture of round-ended cylindrical pellets 18a, flat-ended cylindrical pellets 18b, and spherical pellets 18c. Considerations of symmetry, as well as tests carried out by the present inventor, indicate that the most effective pellet shape is spherical 18c. Ceramic pellets are used as grinding media in size-reduction mills of various types, typically in tumbling mills, and are thus commercially available at a reasonable cost.

In the finished panel 14, pellets 18 are bound by the solidified molten material 16 in a plurality of superimposed rows 20 as viewed in Fig. 1, it being understood that if the panel 14 is disposed horizontally the rows would be adjacent as viewed in Fig. 4. A majority of pellets 18 are each in contact with at least 4 adjacent pellets.

In operation, the panel 14 acts to stop an incoming projectile 12 in one of three modes: centre contact, flank contact, and valley contact, as described above.

Referring now to Fig. 2, a further example of a pellet 18d, is depicted, said pellet having a regular, geometric, prismatic form, with one convex curved surface segment 22.

Fig. 3 shows a pellet 18e having a circular cross-section 24, taken at line AA. The pellet is of satellite form, and is commercially available.

Fig. 4 illustrates a multi-layered, armor panel 26, having a configuration which is particularly suitable for armored clothing. In referring to the following further figures, similar identification numerals are used for identifying similar parts.

An outer, impacting panel 28 of composite armor material is similar to panel 14 described above with reference to Fig. 1. Panel 28 acts to deform and shatter an impacting high velocity projectile 12. Light-weight armor for personal protection is made using a tough, yet hard, thermoplastic resin, for example, polycarbonate or acrylonite-butadiene-styrene.

An inner panel layer 30 is adjacent to outer panel 28, and is advantageously attached thereto. Inner panel layer 30 has a thickness of at least 50% of that of outer impacting panel 28. Inner panel 30 is made of a tough woven material, such as multiple layers of Kevlar®, or a material known by its trade name of Famaston. In a further embodiment, inner layer panel 30 comprises multiple layers of a polyamide netting.

In operation, inner panel 30 causes asymmetric deformation of the remaining fragments 32 of the projectile 12, and absorbs remaining kinetic energy from these fragments by deflecting and compressing them in the area 34 seen in Fig. 1. It is to be noted that area 34 is much larger than the projectile cross-section, thus reducing the pressure felt on the inner side 36 of inner panel 30. This factor is important in personally-worn armor.

Referring now to Fig. 5, there is seen a casting mould 38, used for producing a composite armor material 10 as described above with reference to Fig. 1. The following elevated-temperature method of manufacture is used:

### Step A:

A mould 38 is provided, having a bottom 40, two major surfaces 42, two minor surfaces 44 and an open top 46, wherein the distance between these two major surfaces 42 is 1.2 to 1.8 times the major axis of the pellets 18. For example, 8 mm pellets are used and the distance between major surfaces is 10 mm.

### Step B:

Pellets 18 are inserted into mould 38 to form a plurality of superposed rows 20 of pellets 18, extending substantially along the entire distance between the minor side surfaces 44, and from the bottom 40 substantially to the open top 46.

### Step C:

Mould 38 and the pellets 18 contained therein are incrementally heated, first to a temperature of about 100°C, and then further heated to a temperature of at least 100°C above the flow point of the material to be poured in the mould. For example, aluminium has a flow point of about 540°C, and will require heating the mould, together with ceramic pellets contained therein, to above 640°C. Depending on the alloy being used, it has been found advantageous to heat the mould to a temperature of 850°C.

### Step D:

Molten material 16 is poured into mould 38 to fill the same. A typical pour temperature range for aluminium is 830-900°C. Polycarbonate is poured at between 250-350°C. Advantageously, the surfaces of mould 38 are provided with a plurality of air holes 48, to facilitate the escape of air while molten material 16 is poured therein. During pouring, the pellets 18 are slightly rearranged in accordance with the hydrostatic and hydrodynamic forces exerted upon them by the molten material.

### Step E:

Molten material 16 is allowed to solidify.

### Step F:

Composite armor material 10 is removed from mould 38.

The following embodiment of a method of manufacture includes the use of an epoxy resin to form a themoset matrix. As is known, epoxies can be cast at room temperature and chemically hardened, or their hardening can be accelerated by the application of heat. Epoxy armor is suitable for use on aircraft. Yield strength and Young's modulus are both improved by adding fiber reinforcement.

### Step A:

Mould 38 is provided, having a bottom 40, two major surfaces 42, two minor surfaces 44 and an open top 46, wherein the distance between the two major surfaces 42 is from about 1.2 to 1.8 times the major axis of the pellets 18.

### Step B:

Pellets 18 are inserted into mould 38 to form a plurality of superposed rows 20 of pellets 18 extending substantially along the entire distance between the minor side surfaces 44, and from the bottom 40 substantially to the open top 46.

### Step C:

Liquid epoxy resin is poured into mould 38 to fill the same.

### Step D:

The epoxy is allowed to solidify.

### Step E:

The composite armor material is removed from mould 38.

Table 1 is a reproduction of a test report relating to the aluminium matrix multi-layer panel described above with reference to Fig. 4. Three armor-piercing bullets were fired at close range from an AK-47 assault rifle at a multi-layered panel having a total weight of 34.3 kg/m², a weight low enough for limited use as personally worn armor. The results reported prove the effectiveness of the panel manufactured according to the present invention.

The present embodiments are to be considered in all respects as illustrative and not restrictive, the scope of the invention being indicated by the wording of the appended claims rather than by the foregoing description, and all changes which come within the meaning and range of equivalency of the claims are therefore intended to be embraced therein.

## Claims

1. A composite armor plate for absorbing and dissipating kinetic energy from high velocity, armor-piercing projectiles, said plate comprising a single internal layer of high density ceramic pellets which are directly bound and retained in plate form by a solidified material such that the pellets are bound in a plurality of superposed rows and each of a majority of said pellets is in contact with at least four adjacent pellets, characterised in that the pellets have an Al₂ O₃ content of at least 93% and a specific gravity of at least 2.5, the majority of the pellets each have a major axis of a length in the range of from 3 to 12 mm, the solidified material, and hence the plate, is elastic at a temperature below 250°C, and the weight of said plate does not exceed 45 kg/m².

2. A composite armor plate as claimed in claim 1, wherein the majority of said pellets each has a major axis of a length in the range of from 6 to 10 mm.

3. A composite armor plate as claimed in claim 1, wherein said pellets are of a regular geometric form, having at least one convex curved surface segment.

4. A composite armor plate as claimed in claim 1, wherein said pellets have at least one circular cross-section.

5. A composite armor plate as claimed in claim 1, wherein said pellets are of round-ended cylindrical shape, flat-ended cylindrical shape, or spherical shape.

6. A composite armor plate as claimed in claim 1, wherein said ceramic pellets have a specific gravity of at least 3.

7. A composite armor plate as claimed in claim 1, wherein said pellets have a hardness of 9 on the Mohs scale.

8. A composite armor plate as claimed in claim 1, wherein said solidified material contains at least 80% aluminium.

9. A composite armor plate as claimed in claim 1, wherein said solidified material is a thermoplastic resin.

10. A composite armor plate as claimed in claim 1, wherein said solidified material is an epoxy.

11. A multi-layered armor panel comprising an outer, impact-receiving layer, consisting of a composite armor plate according to claim 1, for deforming and shattering an impacting high velocity, armor-piercing projectile, and an inner layer adjacent said outer layer comprising a tough woven textile material for causing an asymmetric deformation of the remaining fragments of said projectile and for absorbing the remaining kinetic energy from said fragments, said inner layer having a thickness of at least 50% of that of said outer, impact-receiving layer, and said panel being capable of stopping three bullets fired sequentially at a triangular area of said panel, the sides of said triangle being 5 cm each.

12. A multi-layered armor panel according to claim 11, wherein said inner layer is made of Kevlar®.

13. A multi-layered armor panel according to claim 11, wherein said inner layer comprises multiple layers of a polyamide netting.

14. A method for producing a composite armor plate according to claim 1, comprising:
providing a mould having a bottom, two major surfaces, two minor side surfaces and a open top, wherein the distance between said two major surfaces is from about 1.2 to 1.8 times the major axis of said pellets.
inserting said pellets into said mould to form a plurality of superposed rows of pellets extending substantially along the entire distance between said minor side surfaces, and from said bottom substantially to said open top;
incrementally heating said mould and the pellets contained therein to a temperature of at least 100°C above the flow point of the material to be poured in the mould;
pouring said molten material into said mould to fill the same;
allowing said molten material to solidify; and
removing said composite armor plate from said mould.

15. A method as claimed in claim 14, wherein said solidified molten material comprises a casting alloy containing at least 80% aluminium, and said mould is heated to a temperature of at least 850°C.

16. A method as claimed in claim 14, wherein said surfaces of said mould are provided with a plurality of air holes to facilitate the escape of air while said molten material is poured therein.

17. A method for producing a composite armor plate according to claim 1, comprising:
providing a mould having a bottom, two major surfaces, two minor surfaces and an open top, wherein the distance between said two major surfaces is from about 1.2 to 1.8 times the major axis of said pellets;
inserting said pellets into said mould to form a plurality of superposed rows of pellets extending substantially along the entire distance between said minor side surfaces, and from said bottom substantially to said open top;
pouring liquid epoxy resin into said mould to fill the same;
allowing said epoxy to solidify; and
removing said composite armor plate from said mould.

## Patentansprüche

1. Verbundpanzerplatte zum Absorbieren und Ableiten von kinetischer Energie panzerbrechender Projektile mit hoher Geschwindigkeit, wobei die Platte eine einzelne innere Schicht so aus hochdichten Keramikpellets umfaßt, die so durch ein verfestigtes Material direkt verbunden und in Plattenform gehalten werden, daß die Pellets in einer Vielzahl übereinanderliegender Reihen verbunden sind, und jedes einer Mehrzahl der Pellets in Kontakt mit wenigstens vier benachbarten Pellets ist, **dadurch gekennzeichnet,** daß die Pellets einen Al₂O₃- Gehalt von wenigstens 93% und eine relative Dichte von wenigstens 2,5 haben, wobei die Mehrzahl der Pellets jeweils eine Hauptachse einer Länge im Bereich von 3 bis 12 mm hat, das verfestigte Material und damit die Platte bei einer Temperatur unter 250°C elastisch ist und das Gewicht der Platte 45 kg/m² nicht übersteigt.

2. Verbundpanzerplatte nach Anspruch 1, wobei die Merzahl der Pellets jeweils eine Hauptachse einer Länge im Bereich von 6 bis 10 mm hat.

3. Verbundpanzerplatte nach Anspruch 1, wobei die Pellets regelmäßige geometrische Form mit wenigstens einem konvexen gekrümmten Flächensegment haben.

4. Verbundpanzerplatte nach Anspruch 1, wobei die Pellets wenigstens einen kreisförmigen Querschnitt haben.

5. Verbundpanzerplatte nach Anspruch 1, wobei die Pellets zylindrische Form mit runden Enden, zylindrische Form mit flachen Enden oder Kugelform haben.

6. Verbundpanzerplatte nach Anspruch 1, wobei die Keramik-Pellets eine relative Dichte von wenigstens 3 haben.

7. Verbundpanzerplatte nach Anspruch 1, wobei die Pellets eine Dichte von 9 auf der Mohs'schen Skala haben.

8. Verbundpanzerplatte nach Anspruch 1, wobei das verfestigte Material wenigstens 80% Aluminium enthält.

9. Verbundpanzerplatte nach Anspruch 1, wobei das verfestigte Material ein Thermoplastharz ist.

10. Verbundpanzerplatte nach Anspruch 1, wobei das verfestigte Material ein Epoxydharz ist.

11. Mehrschichtige Panzertafel, die eine äußere schlagaufnehmende Schicht, die aus einer Verbundpanzerplatte nach Anspruch 1 besteht, um ein mit hoher Geschwindigkeit auftreffendes panzerbrechendes Projektil zu verformen und zu zertrümmern, sowie eine innere Schicht umfaßt, die an die äußere Schicht angrenzt und festgewebtes Textilmaterial umfaßt, um eine asymmetrische Verformung der restlichen Bruchteile des Projektils zu bewirken und die verbleibende kinetische Energie der Bruchteile zu absorbieren, wobei die innere Schicht eine Dicke von wenigstens 50% der äußeren schlagaufnehmenden Schicht hat, und die Tafel in der Lage ist, drei Geschosse aufzuhalten, die nacheinander auf einen dreieckigen Bereich der Tafel geschossen werden, wobei die Seiten des Dreiecks jeweils 5 cm lang sind.

12. Mehrschichtige Panzertafel nach Anspruch 11, wobei die innere Schicht aus Kevlar® besteht.

13. Mehrschichtige Panzertafel nach Anspruch 11, wobei die innere Schicht mehrere Schichten eines Polyamidnetzes umfaßt.

14. Verfahren zum Herstellen einer Verbundpanzerplatte nach Anspruch 1, das umfaßt:
Bereitstellen einer Form mit einem Boden, zwei Hauptflächen, zwei Nebenseitenflächen und einer offenen Oberseite, wobei der Abstand zwischen den beiden Hauptflächen ungefähr dem 1,2- bis 1,8-fachen der Hauptachse der Pellets entspricht;
Einbringen der Pellets in die Form, um eine Vielzahl übereinanderliegender Reihen von Pellets herzustellen, die sich im wesentlichen über den gesamten Abstand zwischen den Nebenseitenflächen und von dem Boden aus im wesentlichen bis zu der offenen Oberseite erstrecken;
schrittweises Erhitzen der Form und der darin enthaltenen Pellets auf eine Temperatur von wenigstens 100°C über dem Fließpunkt des in die Form zu gießenden Materials;
Gießen des geschmolzenen Materials in die Form, um selbige zu füllen;
Verfestigen des geschmolzenen Materials; und
Entnehmen der Verbundpanzerplatte aus der Form.

15. Verfahren nach Anspruch 14, wobei das verfestigte geschmolzene Material eine Gießlegierung umfaßt, die wenigstens 80% Aluminium enthält, und die Form auf eine Temperatur von wenigstens 850°C erhitzt wird.

16. Verfahren nach Anspruch 14, wobei die Flächen der Form mit einer Vielzahl von Luftlöchern versehen sind, um das Austreten von Luft zu erleichtern, wenn das geschmolzene Material eingegossen wird.

17. Verfahren zum Herstellen einer Verbundpanzerplatte nach Anspruch 1, das umfaßt:
Bereitstellen einer Form mit einem Boden, zwei Hauptflächen, zwei Nebenflächen und einer offenen Oberseite, wobei der Abstand zwischen den beiden Hauptflächen ungefähr dem 1,2- bis 1,8-fachen der Hauptachse der Pellets entspricht;
Einbringen der Pellets in die Form, um eine Vielzahl übereinanderliegender Reihen von Pellets herzustellen, die sich im wesentlichen über den gesamten Abstand zwischen den zwei Nebenseitenflächen und von dem Boden aus im wesentlichen bis zu der offenen Oberseite erstrecken;
Eingießen von flüssigem Epoxydharz in die Form, um selbige zu füllen;
Verfestigen des Epoxydharzes; und
Entnehmen der Verbundpanzerplatte aus der Form.

## Revendications

1. Plaque composite de blindage destinée à absorber et dissiper l'énergie cinétique de projectiles de perçage de blindage à grande vitesse, la plaque comprenant une couche interne unique de pastilles céramiques de haute densité qui sont directement liées et retenues sous forme d'une plaque par un matériau solidifié tel que les pastilles sont liées en plusieurs rangées superposées et chacune des pastilles de la majorité des pastilles est au contact d'au moins quatre pastilles adjacentes, caractérisée en ce que les pastilles ont une teneur en Al₂O₃ au moins égale à 93 % et une densité au moins égale à 2,5, la majorité des pastilles ayant chacune un grand axe dont la longueur est comprise entre 3 et 12 mm, le matériau solidifié, et donc la plaque, étant élastiques à une température inférieure à 250 °C, et le poids de la plaque ne dépassant pas 45 kg/m².

2. Plaque composite de blindage selon la revendication 1, dans laquelle chaque pastille de la majorité des pastilles a un grand axe dont la longueur est comprise entre 6 et 10 mm.

3. Plaque composite de blindage selon la revendication 1, dans laquelle les pastilles ont une forme géométrique régulière, ayant au moins un segment de surface de courbure convexe.

4. Plaque composite de blindage selon la revendication 1, dans laquelle les pastilles ont au moins une section circulaire.

5. Plaque composite de blindage selon la revendication 1, dans laquelle les pastilles ont une forme cylindrique à extrémité arrondie, une forme cylindrique à extrémité plate ou une forme sphérique.

6. Plaque composite de blindage selon la revendication 1, dans laquelle les pastilles céramiques ont une densité au moins égale à 3.

7. Plaque composite de blindage selon la revendication 1, dans laquelle les pastilles ont une dureté égale à 9 sur l'échelle Moh.

8. Plaque composite de blindage selon la revendication 1, dans laquelle le matériau solidifié contient au moins 80 % d'aluminium.

9. Plaque composite de blindage selon la revendication 1, dans laquelle le matériau solidifié est une résine thermoplastique.

10. Plaque composite de blindage selon la revendication 1, dans laquelle le matériau solidifié est une résine époxyde.

11. Panneau multicouche de blindage comprenant une couche externe de réception d'impacts constituée d'une plaque composite de blindage selon la revendication 1, destinée à déformer et briser un projectile de perçage de blindage à grande vitesse à l'impact, et une couche interne adjacente à la couche externe et comprenant un matériau textile tissé tenace destiné à provoquer une déformation asymétrique des fragments restants du projectile et absorber l'énergie cinétique restante des fragments, la couche interne ayant une épaisseur au moins égale à 50 % de celle de la couche externe de réception d'impacts, et le panneau pouvant arrêter trois balles tirées successivement dans une région triangulaire du panneau, les côtés du triangle ayant chacun une dimension de 5 cm.

12. Panneau multicouche de blindage selon la revendication 11, dans lequel la couche interne est formée de "Kevlar".

13. Panneau multicouche de blindage selon la revendication 11, dans lequel la couche interne comporte plusieurs couches de filet de polyamide.

14. Procédé de fabrication d'une plaque composite de blindage selon la revendication 1, comprenant :
la disposition d'un moule possédant un fond, deux surfaces principales, deux petites surfaces latérales et une partie supérieure ouverte, la distance comprise entre les deux surfaces principales étant comprise entre environ 1,2 et 1,8 fois le grand axe des pastilles,
l'insertion des pastilles dans le moule pour la formation de plusieurs rangées superposées de pastilles qui s'étendent pratiquement sur toute la distance comprise entre les petites surfaces latérales et pratiquement du fond à la partie supérieure ouverte,
le chauffage progressif du moule et des pastilles contenues à l'intérieur à une température supérieure d'au moins 100 °C à la température d'écoulement du matériau destiné à être coulé dans le moule,
la coulée du matériau fondu dans le moule afin que celui-ci soit rempli,
la solidification libre du matériau fondu, et
l'extraction de la plaque composite du blindage du moule.

15. Procédé selon la revendication 14, dans lequel le matériau fondu qui se solidifie est un alliage de moulage contenant au moins 80 % d'aluminium, et le moule est chauffé à une température d'au moins 850 °C.

16. Procédé selon la revendication 14, dans lequel les surfaces du moule ont plusieurs trous d'air destinés à faciliter la sortie de l'air lorsque le matériau fondu est coulé dans le moule.

17. Procédé de fabrication d'une plaque composite de blindage selon la revendication 1, comprenant :
la disposition d'un moule ayant un fond, deux grandes surfaces, deux petites surfaces et une partie supérieure ouverte, la distance comprise entre les deux grandes surfaces étant comprise entre 1,2 et 1,8 fois le grand axe des pastilles,
l'insertion des pastilles dans la moule pour la formation de plusieurs rangées superposées de pastilles qui s'étendent pratiquement sur toute la distance comprise entre les petites surfaces latérales, et pratiquement du fond à la partie supérieure ouverte,
la coulée d'une résine époxyde liquide dans le moule afin que celui-ci soit rempli,
la solidification libre de la résine époxyde, et
l'enlèvement de la plaque composite de blindage du moule.
